



US008327524B2

(12) **United States Patent**  
**Brunner**

(10) **Patent No.:** **US 8,327,524 B2**  
(45) **Date of Patent:** **Dec. 11, 2012**

(54) **INDUCTIVE COMPONENT AND METHOD  
FOR THE PRODUCTION THEREOF**

(75) Inventor: **Markus Brunner**, Bessenbach (DE)

(73) Assignee: **Vacuumschmelze GmbH & Co. KG**,  
Hanau (DE)

(\*) Notice: Subject to any disclaimer, the term of this  
patent is extended or adjusted under 35  
U.S.C. 154(b) by 218 days.

(21) Appl. No.: **11/897,875**

(22) Filed: **Aug. 31, 2007**

(65) **Prior Publication Data**

US 2008/0001702 A1 Jan. 3, 2008

**Related U.S. Application Data**

(62) Division of application No. 10/276,653, filed as  
application No. PCT/EP01/03862 on Apr. 5, 2001,  
now Pat. No. 7,265,651.

(30) **Foreign Application Priority Data**

May 19, 2000 (DE) ..... 100 24 824

(51) **Int. Cl.**  
**H01F 7/06** (2006.01)

(52) **U.S. Cl.** ..... **29/606**; 29/602.1; 29/604; 29/605;  
29/607; 336/65; 336/83; 336/90; 336/200;  
336/233

(58) **Field of Classification Search** ..... 29/602.1,  
29/604-607, 840; 336/65, 83, 90-96, 200,  
336/233

See application file for complete search history.

(56) **References Cited**

**U.S. PATENT DOCUMENTS**

3,255,512 A 6/1966 Lochner et al.  
4,059,462 A 11/1977 Masumoto et al.

|               |         |                             |
|---------------|---------|-----------------------------|
| 4,076,861 A   | 2/1978  | Furukawa et al.             |
| 4,201,837 A   | 5/1980  | Lupinski                    |
| 4,305,056 A   | 12/1981 | Mochida et al.              |
| 4,472,334 A   | 9/1984  | Gallimard                   |
| 4,543,208 A   | 9/1985  | Horie et al.                |
| 4,601,765 A   | 7/1986  | Soileau et al.              |
| 4,743,311 A * | 5/1988  | Schultz et al. .... 148/103 |
| 4,923,533 A   | 5/1990  | Shigeta et al.              |
| 4,985,089 A   | 1/1991  | Yoshizawa et al.            |
| 5,038,460 A   | 8/1991  | Ide et al.                  |
| 5,144,745 A   | 9/1992  | Yoshimura et al.            |

(Continued)

**FOREIGN PATENT DOCUMENTS**

DE 502063 7/1930

(Continued)

**OTHER PUBLICATIONS**

Patent Abstracts of Japan, vol. 018, No. 063 (E-1500), Feb. 2, 1984,  
and JP 05 283238, Oct. 29, 1993.

(Continued)

*Primary Examiner* — Paul D Kim

(74) *Attorney, Agent, or Firm* — Buchanan Ingersoll &  
Rooney PC

(57) **ABSTRACT**

Disclosed herein is an inductive component whose soft magnetic core is produced by pouring a casting resin into a mold filled with a soft magnetic alloy powder and by subsequently hardening the casting resin with the alloy powder in order to form a solid soft magnetic core. This technique prevents the surface insulation of the alloy particles from becoming damaged, thereby largely preventing the formation of bulky eddy currents in the resulting soft magnetic cores. This enables a distinct reduction in the electric loss of the inductive component.

**17 Claims, 1 Drawing Sheet**



## U.S. PATENT DOCUMENTS

|                 |         |                      |    |                 |         |
|-----------------|---------|----------------------|----|-----------------|---------|
| 5,160,379 A     | 11/1992 | Yoshizawa et al.     | EP | 0 502 397 A2    | 9/1992  |
| 5,252,148 A     | 10/1993 | Shigeta et al.       | EP | 0435680 B1      | 4/1995  |
| 5,331,730 A     | 7/1994  | Brinn, Jr.           | EP | 0794541 A1      | 9/1997  |
| 5,449,419 A     | 9/1995  | Suzuki et al.        | EP | 0794538         | 5/1998  |
| 5,522,948 A     | 6/1996  | Sawa et al.          | EP | 0 936 638 A2    | 8/1999  |
| 5,594,397 A     | 1/1997  | Uchikoba et al.      | EP | 1 371 434 B1    | 12/2003 |
| 5,751,207 A     | 5/1998  | Poess                | JP | 53055393        | 5/1978  |
| 5,762,967 A *   | 6/1998  | Sagawa et al. ....   | JP | 56-112710       | 9/1981  |
| 5,871,681 A     | 2/1999  | Karino et al.        | JP | 57039516        | 3/1982  |
| 5,973,424 A     | 10/1999 | Engelberger et al.   | JP | 57-122506 A     | 7/1982  |
| 6,001,272 A     | 12/1999 | Ikuma et al.         | JP | 57187357        | 11/1982 |
| 6,028,353 A     | 2/2000  | Nakano et al.        | JP | 59177902        | 10/1984 |
| 6,038,760 A     | 3/2000  | Antoine et al.       | JP | 59179729 A      | 10/1984 |
| 6,103,157 A     | 8/2000  | Behm et al.          | JP | 60-260108 A     | 12/1985 |
| 6,106,376 A     | 8/2000  | Rybak et al.         | JP | 61058450        | 3/1986  |
| 6,189,204 B1 *  | 2/2001  | Shikama et al. ....  | JP | 61172709 A *    | 8/1986  |
| 6,373,368 B1    | 4/2002  | Shikama et al.       | JP | 61210608 A *    | 9/1986  |
| 6,392,525 B1 *  | 5/2002  | Kato et al. ....     | JP | 62-226603       | 10/1987 |
| 6,478,889 B2    | 11/2002 | Kanekiyo             | JP | 62-232103       | 10/1987 |
| 6,663,815 B1    | 12/2003 | Hundt et al.         | JP | 63021807        | 1/1988  |
| 6,682,681 B1    | 1/2004  | Clark et al.         | JP | 63-115313 A     | 5/1988  |
| 6,685,882 B2    | 2/2004  | Deevi et al.         | JP | 1-53404 A       | 3/1989  |
| 6,710,692 B2    | 3/2004  | Kato et al.          | JP | 1-139702        | 6/1989  |
| 6,749,767 B2    | 6/2004  | Mitani et al.        | JP | 02-047812       | 2/1990  |
| 6,750,723 B2    | 6/2004  | Yoshida et al.       | JP | 04021436 A *    | 1/1992  |
| 6,791,445 B2    | 9/2004  | Shibata et al.       | JP | 4-048005 A      | 2/1992  |
| 6,814,776 B2    | 11/2004 | Kanekiyo et al.      | JP | 4165605         | 6/1992  |
| 6,827,557 B2    | 12/2004 | Kim                  | JP | 05-299232       | 11/1993 |
| 7,172,660 B2    | 2/2007  | Song et al.          | JP | 5304018         | 11/1993 |
| 7,175,717 B2    | 2/2007  | Song et al.          | JP | 06-224023       | 8/1994  |
| 7,265,651 B2    | 9/2007  | Brunner              | JP | 8255717         | 10/1996 |
| 7,532,099 B2    | 5/2009  | Brunner              | JP | 83-18542 A      | 12/1996 |
| RE41,269 E      | 4/2010  | Hundt et al.         | JP | 9606715         | 11/1997 |
| 2001/0015239 A1 | 8/2001  | Kanekiyo             | JP | 10-092623       | 4/1998  |
| 2001/0031837 A1 | 10/2001 | Perez et al.         | JP | 10-097913       | 4/1998  |
| 2002/0062885 A1 | 5/2002  | Li                   | JP | 10-208923       | 8/1998  |
| 2002/0124914 A1 | 9/2002  | Kim                  | JP | 2000-182845     | 6/2000  |
| 2003/0156000 A1 | 8/2003  | Brunner              | JP | 2001-068324     | 3/2001  |
| 2004/0045635 A1 | 3/2004  | Bandyopadhyay et al. | JP | 2001-196216     | 7/2001  |
| 2004/0079449 A1 | 4/2004  | Kanekiyo et al.      | JP | 2002-343626 A   | 11/2002 |
| 2004/0089377 A1 | 5/2004  | Deevi et al.         | JP | 2004-063798 A   | 7/2004  |
| 2004/0183643 A1 | 9/2004  | Brunner              | JP | 2004-349585     | 12/2004 |
| 2005/0028889 A1 | 2/2005  | Song et al.          | SU | 338550          | 5/1972  |
| 2005/0034787 A1 | 2/2005  | Song et al.          | WO | WO 00/10755     | 3/2000  |
| 2005/0236071 A1 | 10/2005 | Koshiba et al.       | WO | WO 00/25326     | 5/2000  |
| 2007/0193657 A1 | 8/2007  | Brunner              | WO | WO 00/28556     | 5/2000  |
| 2009/0206975 A1 | 8/2009  | Nuetzel et al.       | WO | WO 00/30132     | 5/2000  |
| 2009/0320961 A1 | 12/2009 | Brunner              | WO | WO 01/18828 A1  | 3/2001  |
| 2010/0194507 A1 | 8/2010  | Brunner              | WO | WO 01/91141 A1  | 11/2001 |
| 2010/0265016 A1 | 10/2010 | Petzold et al.       | WO | WO 02/055749    | 7/2002  |
|                 |         |                      | WO | WO 03/088281 A1 | 10/2003 |

## FOREIGN PATENT DOCUMENTS

|    |                 |         |
|----|-----------------|---------|
| DE | 833493          | 7/1949  |
| DE | 1564643         | 1/1970  |
| DE | 2242958 A1      | 3/1974  |
| DE | 2816173         | 10/1979 |
| DE | 3422281 A1      | 12/1984 |
| DE | 19608891 A1     | 9/1997  |
| DE | 69714103 T2     | 9/1997  |
| DE | 69810551 T2     | 3/1999  |
| DE | 1986069 A1      | 3/2000  |
| DE | 198 37 630 C1   | 5/2000  |
| DE | 19908374 A1     | 9/2000  |
| DE | 199 42 939 A1   | 3/2001  |
| DE | 100 64 024 A1   | 6/2001  |
| DE | 10024824        | 11/2001 |
| DE | 100 31 923 A1   | 1/2002  |
| DE | 19846781        | 9/2002  |
| DE | 103 48 808 B4   | 3/2005  |
| DE | 103 48 810 A1   | 3/2005  |
| DE | 602 05 728 T2   | 3/2006  |
| DE | 10 2006 008 283 | 8/2007  |
| DE | 102006055088 B4 | 6/2008  |
| EP | 0112577         | 7/1984  |
| EP | 0302355         | 2/1989  |
| EP | 0271657         | 11/1989 |
| EP | 0455113         | 11/1991 |

## OTHER PUBLICATIONS

Patent Abstracts of Japan, vol. 010, No. 375 (M-545, Dec. 13, 1986, and JP 61 166902, Jul. 28, 1986).  
 Patent Abstracts of Japan, vol. 012, No. 094 (E-593), Mar. 26, 1988, and JP 62 226603, Oct. 5, 1987.  
 Official Action dated May 30, 2000 for German Patent Publication No. 100 24 824.1-33 (German Language).  
 Notification of Reason for Refusal dated Jun. 29, 2010 for Japanese Patent Application No. 2001-587447.  
 E. Wolfarth: "Ferromagnetic Materials vol. 2,"—Soft Magnetic Metallic Materials—p. 73 (1980).  
 ASM Materials Engineering Dictionary, Edited by J.R. Davis, Davis & Associates, 1992, p. 2002.  
 Official Examination Communication dated Jun. 23, 2009 for Japanese Patent Publication No. JP 2000-565549 (expressed in the German language) and English Translation Certificate of Translation dated Jul. 28, 2009.  
 Kawamura, Yoshihito et al., "Fabrication of Nanocrystalline Fe86Zr7B6Cu1 Soft-Magnetic Compacts with High Saturation Magnetization", J. Applied Physics (ISSN 0021-8979), vol. 76, No. 9, p. 5545-5551, English Abstract, 1994.  
 G.H. Kim et al., "Magnetic properties of FeCuNbSiB nanocrystalline alloy powder cores using ball-milled powder", Journal of Applied Physics, vol. No. 10, Parts 2 and 3, May 15, 2003, pp. 7211-7213.

- D. Nuetzel et al., "Nanocrystalline soft magnetic composite-cores with ideal orientation of the powder-flakes", Journal of Magnetism and Magnetic Materials 196-197, (1999), 327-329.
- Mazaleyrat et al., "Permeability of Soft Magnetic Composites From Flakes of Nanocrystalline Ribbon," IEEE Transactions of Magnetics, vol. 38, No. 5, Sep. 2002, pp. 3132-3134.
- J. Patterson, et al., "Encapsulation of Sensors, Solenoids and Transformers With Engineering Thermoplastics," Proceedings of the Electrical Electronics Insulation Conference, Sep. 18, 1995, pp. 1-6.
- G. Blinne, et al., "Konstruktionskunststoffe fur die Electrotechnik," Systeme und Komponenten, Jun. 1996, pp. 40-42.
- Office Action dated Apr. 22, 2010 for German Patent Application No. 10 2009 038 730.7-24 and English Translation of the same.
- Examination Report dated Feb. 26, 2003 for German Patent Publication No. 101 34 056.7-33 (English Translation and Certificate of Translation dated Nov. 23, 2009).
- Non-Final Office Action dated Jun. 11, 2009 for U.S. Appl. No. 11/663,271.
- Non-Final Office Action dated Sep. 22, 2009 for U.S. Appl. No. 11/663,271.
- Final Office Action dated Oct. 30, 2009 for U.S. Appl. No. 11/343,558.
- Non-Final Office Action dated Apr. 1, 2010 for U.S. Appl. No. 11/343,558.
- Final Office Action dated Oct. 15, 2010 for U.S. Appl. No. 11/343,558.
- Non-Final Office Action dated Aug. 31, 2010 for U.S. Appl. No. 11/878,856.
- Restriction Requirement dated Nov. 4, 2009 for U.S. Appl. No. 11/878,856.
- Non-Final Office Action dated Mar. 22, 2010 for U.S. Appl. No. 11/878,856.
- Restriction Requirement dated Sep. 22, 2010 for U.S. Appl. No. 12/219,615.
- Restriction Requirement dated Apr. 26, 2010 for U.S. Appl. No. 12/486,528.
- Non-Final Office Action dated Jul. 27, 2010 for U.S. Appl. No. 12/486,528.
- Non-Final Office Action dated Sep. 29, 2008 for U.S. Appl. No. 11/343,558.
- Non-Final Office Action dated Apr. 6, 2009 for U.S. Appl. No. 11/343,558.

\* cited by examiner

FIG 1



FIG 2



FIG 3



## 1

INDUCTIVE COMPONENT AND METHOD  
FOR THE PRODUCTION THEREOF

This application is a divisional of U.S. patent application Ser. No. 10/276,653 filed on Mar. 25, 2003, U.S. Pat. No. 7,265,651, which is the U.S. national phase of International Application No. PCT/EP01/03862 filed on Apr. 5, 2001, which claims priority to German Patent Application No. 100 24 824.1 filed on May 19, 2000, the contents of which are incorporated by reference herein.

## BACKGROUND

## 1. Field

Disclosed herein is an inductive component having at least one coil and a soft magnetic core made from a ferromagnetic material. Also disclosed are methods for producing inductive components in particular, which have a soft magnetic core that consists of a powder composite.

## 2. Description of Related Art

Soft magnetic powder composites as pressed magnetic cores have been known for a long time.

Firstly, pressed powder composites made from iron powder are known. A permeability area of approximately 10 to 300 can be covered quite well using this magnetic core. The saturation flux density, which can be obtained using these magnetic cores, is at approximately 1.6 tesla. The application frequencies are generally below 50 kHz due to the size of the comparatively low resistivity and the iron particles.

Pressed powder composites made from soft magnetic crystalline iron aluminum silicon alloys are known as well. Application frequencies exceeding 100 kHz can be reached with these composites due to the comparatively higher resistivity.

Saturation flux densities and permabilities, which are particularly good, can be achieved using powder composite materials, which are based on crystalline mume metals. Permeabilities reaching up to 500 can be achieved via an exact allocation of the nickel content allowing for application frequencies exceeding 100 kHz due to the comparatively minor remagnetizing losses.

However, these three known powder composites can only be processed into very simple geometric forms, as the available press technologies only allow for a limited range. In particular, only toroids and/or pot cores can be produced.

To avoid this disadvantage, an injection molding method was presented in DE 198 46 781 A1, in which nano-crystalline alloys are incorporated into an injection molding capable plastic, and subsequently processed into soft magnetic cores by means of an injection molding method.

It became apparent, however, that the injection molding approaches, which initially seemed to be quite promising, had limitations. A major disadvantage consisted in the alloy particles of the alloy powder made from amorphous or nano-crystalline alloys being exposed to extreme mechanical loads particularly while being injected into the deployed tools. This generally led to damages of the alloy particles' surface insulation. The alloy particles' damaged surface insulations in turn leads to increased remagnetizing losses due to bulky eddy currents in the produced soft magnetic cores.

An additional problem concerning the injection molding method consists in the constancy of the coils' insulation with respect to the soft magnetic core. The mold, which is equipped with coils during the production process, acts rather like an abrasive due to the presence of alloy particles, which are integrated therein, which leads to increased damages of the coils' insulation. Increased serious damage occurs in par-

## 2

ticular, when using coils consisting of copper wires that are insulated with lacquer, or copper strands that are insulated with lacquer.

Furthermore, the need for very expensive injection molding molds, the production of which is very costly, is a disadvantage of the injection molding method.

## SUMMARY

One problem to be solved herein therefore consists in providing an inductive component having at least one coil and a soft magnetic core made from a ferro-magnetic powder composite, which can be produced in a simple manner, and whereby a damage of the insulations to the coils will be avoided as much as possible during the manufacturing process, and where the alloy powder will not be exposed to any, or only to non-critical mechanical loads, during processing.

Furthermore, the new inductive composite and the manufacturing method in connection thereto should not have to do without the advantages of the injection molding method. In particular, it should be possible to make inductive components, whose soft magnetic cores can have almost any shape, and whose volume utilization can be optimized.

As described herein, certain embodiments achieve one or more of these objectives by means of an inductive component having at least one coil and one soft magnetic core made from a ferro-magnetic powder composite, which contains a powder composite consisting of an alloy powder made from an amorphous or nano-crystalline alloy and a casting resin.

In an embodiment as disclosed a method for producing an inductive component having at least one coil and a magnetic soft core, comprising: (a) providing a mold, the at least one coil, an alloy powder, and a casting resin formulation; (b) arranging the at least one coil in the mold; (c1) either: (c1a) soft discharging the alloy powder into the mold, and soft discharging the casting resin formulation into the mold; or (c1b) mixing the alloy powder and the casting resin formulation to produce a mixed casting resin formulation, and soft discharging the mixed casting resin formulation into the mold; (c2) aligning particles of the alloy powder during or after placement of the alloy powder of the mixed casting resin formulation into the mold by creating a magnetic field; and (d) curing the casting resin formulation or the mixed casting resin formulation.

In another embodiment is disclosed an inductive component produced by this method.

In another embodiment is disclosed inductive component, comprising at least one coil and a magnetic soft core made from a ferromagnetic powder composite; said ferromagnetic powder composite comprising an alloy powder from a nano-crystalline alloy and a casting resin and said at least one coil being embedded in said ferromagnetic powder composite, whereby the alloy powder's portion in the powder composite exceeds 55 percent by volume.

## BRIEF DESCRIPTION OF DRAWINGS

The invention method and apparatus disclosed herein shall be explained by means of three embodiment samples and the attached illustration. The following shall be shown:

FIG. 1 is a schematic diagram showing a cross sectional view of an inductive component in accordance with a first embodiment disclosed herein;

FIG. 2 is a schematic diagram showing a cross sectional view of an inductive component in accordance with a second embodiment disclosed herein; and

FIG. 3 is a schematic diagram showing a cross sectional view in accordance with a third embodiment disclosed herein.

#### DETAILED DESCRIPTION OF SPECIFIC EMBODIMENTS

Nano-crystalline alloys are typically used for the alloy powders, as was described in detail for instance in EP 0 271 657 A2 or in EP 0 455 113 A2. Such alloys are typically manufactured by means of the melt spinning technology in form of thin alloy strips, which are amorphous initially, and which are subjected to a heat treatment in order to obtain the nano-crystalline structure. However, amorphous cobalt base alloys can also be used.

In a particular embodiment, the alloys are milled into alloy powders having an average particle size of <2 mm. Thicknesses ranging from 0.01 to 0.04 mm, and measurements of the two other dimensions ranging from 0.04 to 1.0 mm, are most advantageous.

In a particular embodiment, the surfaces of the alloy particles are oxidized in order to achieve an electrical insulation of the alloy particles among themselves. This can be achieved on the one hand by oxidizing the ground alloy particles in an atmosphere, which contains oxygen. The surface oxidation can also be produced by means of the oxidation of an alloy strip before grinding it to an alloy powder.

In certain embodiments, alloy particles could be coated with a plastic, for instance a silane or metal alkyl composite, for a continued improvement of the insulation of the alloy particles among each other, whereby the coating will be performed for 0.1 to 3 hours at a temperature ranging between 80° C. and 200° C. This method "burns" the coating "into" the alloy particles.

In certain embodiments, polyamides or polyacrylates are used as casting resins, whereby the exact procedures will be discussed further below on the basis of the manufacturing method in accordance with this invention.

The inductive components, which were thus manufactured, can show saturation magnetizations  $B_5 \geq 0.5$  and permeabilities  $\mu$  between 10 and 200.

The method described herein for the production of an inductive component having at least one coil and one soft magnetic core made from a ferro-magnetic powder composite is characterized in its first embodiment by the following:

- Providing a mold, an alloy powder and a casting resin formulation;
- Filling the mold with an alloy powder;
- Filling the casting resin formulation in the mold; and
- Curing the casting resin formulation.

In an alternative embodiment, the method for producing an inductive component having at least one coil and one soft magnetic core made from a ferro-magnetic powder composite is characterized by the following steps:

- Providing a mold, an alloy powder and a casting iron formulation;
- Mixing the alloy powder and the casting resin formulation into a casting resin powder formulation;
- Filling the casting resin powder formulation into the mold; and
- Curing the casting resin powder formulation.

This method avoids or minimizes the exposure of the alloy particles to a mechanical load during the manufacturing process, in contrast to the injection molding process, which has been described with respect to DE 198 49 781 A above. Furthermore, the insulation coating, which was applied to the coil wires, will not be damaged particularly when using a mold, which was equipped with a prefabricated coil, since

filling the casting resin formulation or the casting resin powder formulation, of which the viscosity is preferably as low as possible, in the mold does not damage them due to the soft discharge of the formulation. Casting resin formulations having viscosities of a few milli Pascal seconds are preferred in particular.

In an additional embodiment disclosed herein it has been particularly advantageous, particularly with respect to achieving a considerable filling level in the mold, to mix the alloy powder with the casting resin formulation before filling the mold. A small amount of excess casting resin formulation can be used in this embodiment, which benefits the fluidity of the casting resin powder formulation then created. The mold will be made to vibrate by means of a suitable device, for instance by means of a compressed air vibrator, which will thoroughly mix the casting resin formulation and thus fluidize it. The casting resin formulation will be degassed at the same time.

The alloy powder deposits itself in the mold without any difficulties, since the alloy powder features a rather high density as compared with the casting resin, so that the used casting resin excess can be collected in a feeder for instance, which can be removed once the powder composite has hardened.

Inductive components can be produced in one pass due to the use of molds, which are already equipped with prefabricated coils, without a subsequent labor-intensive "wrapping" or application of prefabricated coils onto partial cores, and without a subsequent assembly of the partial cores to complete cores being required.

The mold, which is filled with the alloy powder and the casting resin formulation, or which was filled with a prefabricated casting resin formulation, will continue to be used as the casing of the inductive composite in a preferred embodiment disclosed herein. This means that the mold serves as a "lost casing" in this embodiment of the present invention. This approach provides for a particularly effective and cost-efficient method, which brings with it significant simplifications particularly in contrast to the injection molding process, which had been discussed at the beginning. A mold will always be required for the injection molding process, the production of which is very expensive and costly in addition thereto, and which can never serve as "lost casting".

In the injection molding process the manufactured component or the manufactured soft magnetic core made from a powder composite will always have to be removed from the mold, which is very costly and which leads to extended production times.

In certain embodiments, polymer components, which were mixed with a polymerization initiator (starter), are typically used as casting resin formulations. Methacrylic acid methacrylic esters are considered as polymer components in particular. However, other polymer components, for instance lactame, can be used as well. The methacrylic acid methacrylic esters are polymerized into polyacrylics after having been cured. In an analogous manner, lactame will be polymerized into polyamides via a poly addition reaction.

In particular embodiments, dibenzoyl peroxide can be used as a polymerization initiator, as well as 2,2'-azo isobutyric acid dinitrile, for instance.

However, other polymerization processes of the known casting resins are also possible, such as for instance polymerizations, which are triggered via light or UV radiation that, in other words, largely manage without polymerization initiators.

The alloy particles are aligned during and/or after the filling of the mold with the alloy powder by means of the creation

## 5

of a magnetic field in a particularly preferred embodiment. This can take place particularly when using molds, which have already been equipped with a coil, by means of directing a current through the coil and the accompanying magnetic field. The alloy particles are aligned by means of the creation of magnetic fields, which effectively show field strengths exceeding 10 A/cm.

It is particularly advantageous to align the alloy particles, which are shape anisotropic, along the magnetic field lines, which exist in the subsequently operated inductive component. A significant reduction of the losses and an increase of the permeability of the soft magnetic cores and thus the inductivity of the inductive component can be achieved by aligning the alloy particles by means of their "long" axis parallel to the magnetic field lines.

To obtain higher permeabilities of the soft magnetic core, it is advantageous, when using casting resin powder formulations, to create a magnetic field already at the point of filling the casting resin powder formulation together with the coil, which is lying in the mold, which will act in the direction of the magnetic current thus directing the alloy particles. The mold will be vibrated after having been completely filled, which for instance may take place by means of a compressed air vibrator, and the magnetizing stream will be turned off subsequently. The resulting inductive component will be removed from the form after the final curing of the casting resin formulation.

FIG. 1 shows inductive component 10. Inductive component 10 consists of soft magnetic core 11 and coil 12, consisting of relatively thick copper wire including a few coils. FIG. 1 shows component 10 during its production. Component 10 is brought into mold 1a, which in this case consists of aluminum.

FIG. 2 also shows inductive component 20, consisting of a soft magnetic core made from powder composite 21 in which layer coil-bobbin coil former 22 was brought in. Layer coil-bobbin coil former 22 is connected to pins 23 at its coil ends, which protrude from soft magnetic core 21, and serve to connect to a base plate, for instance a conductor board. Inductive component 20 in FIG. 2 is shown as well as in FIG. 1 during its production. This means that inductive component 20 is shown here in mold 1b, into which the powder composite is poured.

FIG. 3 also shows an inductive component as in FIGS. 1 and 2. Inductive component 30 shown here consists of soft magnetic core 31 made from a powder composite into which in turn layer coil-bobbin coil former 32 was brought in. Layer coil-bobbin coil former 32 is connected at its coil ends with connection pins 33, which protrude from mold 1c, which also serves as casing 34.

The following features are identical in all three embodiments shown in FIGS. 1 through 3, as long as not explicitly specified otherwise.

The base material for the powder composite in all three of the illustrated embodiments of the invention consists of an alloy, which is composed as follows:  $Fe_{73.5}Cu_1Nb_3Si_{15.5}B_7$ , which has been produced in accordance with the known quick set technology process as thin metal strips. It is noted again that these manufacturing processes are explained in detail for instance in EP 0 271 657 A2. These alloy strips are subsequently heat treated for purposes of setting the nano-crystalline structure under hydrogen or in a vacuum at a temperature of approximately 556° C. The alloy strips are crushed in a grinder to achieve the desired final fineness after this crystallization treatment. The thickness of the alloy particles, which typically resulted from this process ranged from 0.01 to 0.04 mm, and the measurements of the two other dimensions ranged from 0.04 to 1.0 mm.

The alloy particles, which were created in this manner, and which are occasionally called flakes, are now provided with a

## 6

surface coating in order to improve their dynamic magnetic characteristics. First of all, a specific surface oxidation of the alloy particles by means of a heat treatment at temperatures ranging from 400° C. to 540° C. for a duration ranging from 0.1 to 5 hours were performed for this purpose. The alloy particles' surface was covered with an abrasion-proof layer consisting of iron and silico-oxide with a typical layer thickness of approximately 150 to 400 nm after the heat treatment.

The alloy particles were coated with silane in a fluidized bed coater following the surface oxidation. The layer was subsequently annealed at temperatures ranging from 80° C. to 200° C. for 0.1 to 3 hours.

The alloy particles, which were prepared in this manner, were subsequently filled in molds 1a or 1b in the embodiments of the invention, which are illustrated in FIGS. 1 and 2.

Molds 1a or 1b, which are made of aluminum, featured a suitable isolation coating at their interior walls so that the removal of inductive components 10 or 20 from the mold was uncomplicated. Electric currents were conducted through coils 12 or 22 so that the alloy particles aligned themselves with their "long axis" parallel to the thus created magnetic field, which was approximately 12 A/cm.

Subsequently, a casting resin formulation was introduced into the respective molds, which were filled with alloy powder in the embodiment examples herein, which are illustrated in FIGS. 1 and 2.

A thermoplastic methacrylate formulation was filled together with a silane bonding agent into the embodiment shown in FIG. 1. This thermoplastic methacrylate formulation was composed of the follows:

100 g methacrylic acid/methacrylic esters  
30 2 g methacrylic trimethoxy silane  
6 g dibenzoyl peroxide and  
4.5 g N,N-dimethyl-p-toluidine

Likewise, a thermoplastic methacrylates formulation together with a silane bonding agent was filled in the embodiment illustrated in FIG. 2, whereby this methacrylate formulation was composed as follows:

100 g methacrylic acid/methacrylic esters  
2 g methacrylic trimethoxy silane  
10 g diglycoldimethacrylate  
40 6 g dibenzoyl peroxide and  
4.5 g N,N-dimethyl-p-toluidine

The above-mentioned chemical components were dissolved one after the other in methacrylic ester in both embodiments. The final mixture was clear like water in both cases. It was subsequently poured into molds 1a and 1b. The casting resin formulations were cured in both cases at room temperatures within approximately 60 minutes. Post-curing at approximately 150° C. took place after that for an additional hour.

When filling molds 1a or 1b with the alloy powder it proved to be practical to vibrate molds 1a or 1b during the filling process, in order to thus densify the alloy powder. In both cases volume shares of up to 55 vol % of the alloy powder could be easily obtained in the powder composite by means of this process.

55 A hot curing thermoplastic methacrylate formulation was used in the embodiment shown in FIG. 3, and which is composed of the following:

100 g methacrylic acid methacrylic esters  
0.1 g 2,2'-azo isobutanoic acid dinitril.

This casting resin formulation was filled into mold 1c, as shown in FIG. 3, and cured within 15 hours at a temperature of approximately 50° C. Since mold 1c in FIG. 3 was used as "lost casing", i.e., since it was used as casing 34 for the inductive component after the production process, the use of a hot curing casting resin formulation had proven to be particularly beneficial as it succeeded in creating a particularly intense and superior contact between mold 1c, which is made of plastic, and the powder composite.

This casting iron formulation was then post cured at a temperature of approximately 150° C. for one hour.

It is noted that the afore-mentioned casting resin formulations only serve as examples. A large variety of other casting resins can be used, of which the chemical cross-links differ from the above-mentioned formulations.

For the sake of completeness it is noted that the above-mentioned formulations were polymerized and that dibenzoyl peroxide or 2,2'-azo isobutanoic acid dinitril was used as initiator substances. However, it is specifically possible to make do without a special initiator substance, and to polymerize monomer components, i.e. chemical substances such as the methacrylic acid methacrylic ester mentioned here, by means of ultraviolet light.

The toughness or the impact resistance of the created powder composite can be increased in particular by mixing in methacrylic trimethoxy silane or diglycoldimethacrylate and other chemical substances.

In particular, melts created from 8-caprolactam and phenylisocyanate can be used when using thermoplastic polyamides; thus a melt created from 100 g 8-caprolactam and 0.4 g phenylisocyanate, which were mixed at a temperature of 130° C., has proven suitable in subsequent tests. This melt was then filled into a form, which had been preheated to 130° C. The curing of caprolactam to a polyamide occurred within approximately 20 minutes. Post-curing at higher temperatures was generally not required when using this process.

Naturally, another lactam can be used instead of caprolactam, such as for instance laurinlactam, together with an appropriate bonding phase. However, process temperatures exceeding 170° C. will be required for processing laurinlactam.

Inductive components having soft magnetic cores were made from ferro-magnetic powder composites using the above-mentioned casting resin formulations, which showed much lower remagnetizing losses than the inductive components which were produced in an analogous manner using the injection mold process. Thus, for instance, remagnetizing losses ranging from 200 to 600 w/kg were reached using injection molded components at 100 kHz and a shakedown of 0.1 tesla.

By contrast, losses under 100 w/kg could be reached using the inductive component and the accompanying manufacturing process under the same magnetizing conditions, whereby the filling degrees of the injection molded inductive components and of the inductive component, which has been produced by means of the process disclosed herein, were almost identical.

The invention having been described above with reference to certain specific embodiments thereof, it will be recognized that these embodiments do not limit the scope of the appended claims.

The invention claimed is:

1. A method for producing an inductive component having at least one coil and a magnetic soft core, comprising:
  - (a) providing a mold, the at least one coil, an alloy powder, and a casting resin formulation;
  - (b) arranging the at least one coil in the mold;
  - (c1) either:
    - (c1a) soft discharging the alloy powder into the mold, and soft discharging the casting resin formulation into the mold; or
    - (c1b) mixing the alloy powder and the casting resin formulation to produce a mixed casting resin formulation, and soft discharging the mixed casting resin formulation into the mold;

(c2) aligning particles of the alloy powder during or after placement of the alloy powder of the mixed casting resin formulation into the mold by creating a magnetic field created by an electrical current that is directed through the at least one coil when the coil is in the mold; and

(d) curing the casting resin formulation or the mixed casting resin formulation without removing the at least one coil from the mold, so that the coil becomes part of the cured inductive component.

2. The method according to claim 1, comprising:

- (a) providing the mold, the at least one coil, the alloy powder, and the casting resin formulation;
- (b) arranging the at least one coil in the mold;
- (c1) soft discharging the alloy powder into the mold; and soft discharging the casting resin formulation into the mold;
- (c2) aligning the particles of the alloy powder during or after placement of the alloy powder into the mold; and
- (d) curing the casting resin formulation.

3. The method in accordance with claim 2, wherein the at least one coil is coated with an insulation film.

4. The method in accordance with claim 2, wherein the mold is used as a casing of the inductive component.

5. The method in accordance with claim 2, wherein the casting resin formulation consists of polymer components and a polymerization initiator.

6. The method in accordance with claim 5, wherein methacrylic acid methyl ester is used as a polymer component.

7. The method in accordance with claim 6, wherein dibenzoyl peroxide is used as a polymerization initiator.

8. The method in accordance with claim 6, wherein 2,2'-azoisobutanoic acid dinitril is used as a polymerization initiator.

9. The method in accordance with claim 2, wherein the created magnetic field has a field strength of at least 10 A/cm.

10. The method according to claim 1, comprising:
 

- providing the mold, the at least one coil, the alloy powder, and the casting resin formulation;
- arranging the at least one coil in the mold;
- mixing the alloy powder and the casting resin formulation to produce a mixed casting resin formulation;
- soft discharging the mixed casting resin formulation into the mold;
- aligning particles of the alloy powder during or after placement of the mixed casting resin formulation into the mold; and
- curing the mixed casting resin formulation.

11. The method in accordance with claim 10, wherein the at least one coil is coated with an insulation film.

12. The method in accordance with claim 10, wherein the mold is used as a casing of the inductive component.

13. The method in accordance with claim 10, wherein the casting resin formulation consists of polymer components and a polymerization initiator.

14. The method in accordance with claim 13, wherein methacrylic acid methyl ester is used as a polymer component.

15. The method in accordance with claim 14, wherein dibenzoyl peroxide is used as a polymerization initiator.

16. The method in accordance with claim 14, wherein 2,2'-azoisobutanoic acid dinitril is used as a polymerization initiator.

17. The method in accordance with claim 1, wherein the created magnetic field has a field strength of at least 10 A/cm.